

## UNITED STATES PATENT OFFICE

1,964,204

PRESS AND WIRE FOR INCANDESCENT  
LAMPS, RADIO TUBES, AND THE LIKEHerbert C. Jennison, Bridgeport, Conn., assignor  
to The American Brass Company, Waterbury,  
Conn., a corporation of ConnecticutNo Drawing. Application March 6, 1931,  
Serial No. 520,721

3 Claims. (Cl. 176—36)

This invention relates to an improved copper wire for use as the lead in wires to be welded to the wires passing through the glass seal in incandescent lamps, radio lamps or tubes, and like devices, and has for an object to provide an improved copper wire which will more readily and effectively operate for the automatic electric welding of these lead in wires to the wires passing through the glass seal, and will give a better and stronger connection which will not become brittle in subsequent manufacturing operations for the lamp, tube or the like.

It is a more specific object of the invention to provide a special manganese deoxidized copper wire which will contain sufficient manganese to secure the above noted results.

With the foregoing and other objects in view the invention consists in certain novel features as will be more fully disclosed and pointed out hereinafter.

20 In all lamps of the above description (the term lamp being used to include radio tubes and similar devices as well as incandescent lamps) the lead in wires are of copper, and practically the universal practice in manufacturing is to automatically 25 electrically weld these lead in wires to the metal wires that pass through the glass seal in the lamp or tube. It has heretofore been common practice to use standard electrolytic copper wire for these lead in wires. This wire welds quite satisfactorily but it contains a certain amount of oxygen in the form of cuprous oxide distributed throughout the copper. This oxygen content may be 0.10 percent or less. In certain operations in manufacturing some of the lamps it is necessary 30 to heat the copper lead in wires in an atmosphere of hydrogen or other reducing gases, and during these operations these reducing gases react with the oxygen in the electrolytic copper wire and reduce the cuprous oxide, or in other words the 35 copper is "gassed" as this action is termed by the trade. This is very objectionable because electrolytic copper that has been heated in hydrogen or other reducing atmospheres and becomes "gassed" is very brittle and has very little strength, 40 and therefore is practically worthless after this annealing in reducing atmospheres. In an attempt to overcome these objections I have found that wires prepared from certain deoxidized copper behave very satisfactorily in the automatic 45 electric welding and in the subsequent annealing 50 in hydrogen and other reducing gases.

In producing deoxidized copper wire the copper is first melted in a crucible or suitable furnace and after it is thoroughly melted a deoxidizer 55 is added. Various deoxidizers such as phosphor-

ous, silicon, aluminum and other deoxidizers well known to the art have been used. The deoxidizer combines with the oxygen in the molten copper and thus frees the copper of oxygen as the oxygen combines with the deoxidizer and slags off leaving the copper free from oxygen. The metal is then poured into bars suitable for rolling, drawing etc. into wire.

On experimentation, however, it was found that copper deoxidized with various deoxidizers such for example as phosphorus, silicon and others made very unsatisfactory welds, particularly when used in the automatic welding machine for welding lead in wires to the wires leading through the glass seal in electric lamps, tubes and the like. I discovered, however, that manganese deoxidized copper wire in which a certain amount of manganese remained in the wire was very satisfactory both from the standpoint of manipulation in the welding operation and the strength of the finished weld as well as standing up under subsequent manufacturing operations for the lamps, and as having the required high electric conductivity.

In producing this wire the melting, pouring and casting of the deoxidized copper is so conducted that not only is the copper deoxidized but some manganese is retained in the copper. My experiments at the present time indicate that the preferred amount of manganese is from about 0.01 percent to about 0.10 percent, and that for best results about 0.075 percent of manganese should remain in the copper. Smaller amounts of manganese will give fairly satisfactory results under certain conditions as will also somewhat greater amounts, but I have found that about these percentages of manganese retained in the deoxidized copper wire will give the most satisfactory results. If the manganese content is much higher than 0.075 percent the electrical conductivity of the wire is lowered beyond the point which is satisfactory, as high electrical conductivity is very desirable in lead in wires to lamps in order to keep the resistance as low as possible. If a consumer is willing to use a wire having a lower conductivity, a higher manganese content may be used.

With the manganese content lower than 0.075 percent there is greater danger of the wire not being properly deoxidized and also greater danger of its not behaving properly in the automatic welding machine, but tests indicate that a manganese content in the deoxidized copper wire as low as 0.001 percent, and as high as 0.25 percent would be fairly satisfactory the higher content

being capable of use where a lower electrical conductivity would be satisfactory. For best all round results about 0.075 percent manganese in the deoxidized copper wire appears to be the most satisfactory, although this manganese content may be varied depending upon conductivity requirements. This assures that the copper is properly deoxidized so that we will not have the action of "gassing" with its objectionable effects in subsequent manufacturing operations.

The presence of the manganese prevents the absorption of oxygen during the welding operation, and also makes the metal weld more readily. It has further been found that this manganese deoxidized copper wire containing substantially the amounts of manganese mentioned behaves in a peculiar manner in the welding operation, in that the bead of melted metal formed at the weld remains concentric with the wire, whereas in welding other types of deoxidized copper wire the bead is formed eccentrically in this class of work. This is very important as giving a better and more reliable weld, particularly as these automatic welding machines operate with the wires in a horizontal position.

Having thus set forth the nature of my invention, what I claim is:

1. In combination a press for incandescent lamps, radio tubes and the like, a wire sealed in said press with one end adjacent thereto, and a lead-in wire composed of copper containing manganese in amount from 0.001 percent to approximately 0.25 percent welded to said adjacent end. 80
2. In combination a press for incandescent lamps, radio tubes and the like, a wire sealed in said press with one end adjacent thereto, and a lead-in wire composed of copper containing manganese in amount from approximately 0.010 percent to 0.10 percent welded to said adjacent end. 85
3. In combination a press for incandescent lamps, radio tubes and the like, a wire sealed in said press with one end adjacent thereto, and a lead-in wire composed of copper containing approximately 0.075 percent manganese welded to 95 said adjacent end.

HERBERT C. JENNISON.

30

105

35

110

40

115

45

120

50

125

55

130

60

135

65

140

70

145

75

150